

# UNITED STATES PATENT OFFICE.

JAMES C. CLEARY, OF CHICAGO, ILLINOIS, ASSIGNOR TO MICHAEL W. BORDERS, OF CHICAGO, ILLINOIS.

## PROCESS OF TANNING LEATHER.

1,107,759.

Specification of Letters Patent. Patented Aug. 18, 1914.

No Drawing.

Application filed October 30, 1911. Serial No. 657,644.

To all whom it may concern:

Be it known that I, JAMES C. CLEARY, a citizen of the United States, and a resident of Chicago, in the county of Cook and State 5 of Illinois, have invented a certain new and useful Improvement in Processes of Tanning Leather, of which the following is a specification.

This invention relates to a process of tanning hides and relates particularly to a 10 process of tanning hides with liquor produced by the destructive distillation of lignite of the cretaceous age or period, as fully set forth and described in an application for 15 U. S. Letters Patent heretofore filed by George Kimball on the 24th day of April, 1908, Serial Number 428,939, as well as in the later application filed by said Kimball on the 30th of June, 1913, Serial No. 776,640.

The process set forth in the aforesaid applications is briefly as follows:—The hides to be tanned are first pickled, in substantially the usual way, and are then immersed until 20 properly tanned in a bath consisting of a liquor such as is obtained by the destructive distillation of a lignite coal of the cretaceous age or period which occurs and is produced in several counties in the State of Arkansas, including the county of Ouachita 25 in said State and described on page 28 of a work known as "*The Minerals and Rocks of Arkansas*," published by F. L. Harvey, B. S. in 1886. For purposes of convenient reference, the particular lignite from which the 30 tanning liquor is obtained for use in practising the process of the aforesaid application will be referred to hereinafter as "Ouachita" lignite. This tanning liquor is obtained by the destructive distillation of 35 the lignite for a period of from seven to ten 40 hours at temperatures of from 300° to 450° F., the distillation being performed in any usual form of retort. The distillate consists principally of two distinct products, a watery 45 liquor and an oil, which separate by gravity, the watery liquor being the heavier and soon settling when the full liquor is allowed to stand, so that it can be readily drawn off from the oil. The watery distillate carries 50 in solution certain of the higher phenols, and this watery distillate alone may be used or the full liquor, containing the oil, may be used, the oily distillate operating to impart 55 a dark color and a distinctive odor to the leather.

It has been found that, in practising the process set forth in the aforesaid application, the leather produced thereby is too porous for ordinary uses, making it necessary that it be subjected to special treatment to impart the desired density and firmness thereto. On the other hand, it is well known by persons skilled in the tanning art that hides tanned by means of usual tanning agents, such as extract of hemlock, oak, quebracho, alum, chromium, and the like are hard and brittle and break very easily, if bent, making it necessary to treat them with grease to render the leather soft and pliable.

I have discovered that by using as a tanning agent a mixture of the aforesaid liquor distilled from "Ouachita" cretaceous lignite and one of the well known tanning agents, as hemlock extract or its equivalent, 70 and for some hides, particularly sheepskins, a mixture of "Ouachita" cretaceous lignite distillate and a mineral tanning agent, as alum, chromium, or an equivalent thereof, a leather will be produced having the density 75 and firmness of leather tanned with usual vegetable or mineral tannages now in common use, and the softness and pliability of leather tanned with the "Ouachita" cretaceous lignite distillate, and that the tanning process 80 requires only from one quarter (1) to one-third (1/3) of the time required for tanning similar hides by present processes. For example, it requires from three to four months 85 to tan sole leather, harness leather and the like by present methods, whereas, by my improved process leather of the same character and believed to be of superior quality can be produced in from four to five weeks.

In the practice of my invention, the hides 90 are first pickled, substantially in the usual way, and are then immersed in a bath consisting of a mixture of liquor produced by the destructive distillation of "Ouachita" 95 cretaceous lignite and a usual tanning agent, 100 preferably one which contains tannic acid, as extract of hemlock, oak, quebracho. For most purposes, I prefer to mix said tannages in the proportions of about eleven (11) pounds of said extract to forty (40) 105 gallons of the liquor distilled from "Ouachita" cretaceous lignite. Also, I find that the best results are obtained by adding the extract—hemlock, oak or the like—gradually, increasing the proportion and effect 110

of said extract as the process progresses. Thus, at the beginning of the process, I add to the "Ouachita" cretaceous lignite distillate (40 gallons) only one (1) pound of 5 the extract; at the beginning of the second week, three (3) pounds; at the beginning of the third week, three (3) pounds; and, at the beginning of the fourth week, four (4) pounds. I do not, however, wish to limit 10 myself to the exact proportion of extract and of "Ouachita" lignite distillate specified, as excellent results may be obtained by varying the proportions thereof within a considerable range.

15 The length of time required for tanning different hides will vary, but skilled operators can readily ascertain by examination when the hides are thoroughly tanned.

When the tanning process is completed, 20 the hides are removed from the liquor and subjected to any desired finishing process.

I claim:

1. The process of tanning hides which 25 consists in first preparing the hides in any usual manner, and in then soaking them in a bath consisting of liquor such as is produced by the destructive distillation of "Ouachita" cretaceous lignite and a usual tanning extract or agent, substantially as 30 described.

2. The process of tanning hides which 35 consists in first preparing the hides in any usual manner, and in then soaking them in a bath consisting of liquor such as is produced by the destructive distillation of "Ouachita" cretaceous lignite and a usual

tanning extract or agent in substantially the proportions of forty (40) gallons of "Ouachita" distillate to eleven (11) pounds of extract, substantially as described.

40

3. The process of tanning hides which consists in first preparing the hides in any usual manner, and in then soaking them in a bath consisting of liquor such as is produced by the destructive distillation of 45 "Ouachita" cretaceous lignite and a usual tanning extract or agent, the extract being added gradually as the tanning process progresses, substantially as described.

4. The process of tanning hides which 50 consists in first pickling the hides in the usual manner, then soaking them in a bath consisting of liquor such as is produced by the destructive distillation of Ouachita cretaceous lignite to which a tanning extract is added in about the proportion of 55 forty gallons of such distillate to one pound of extract, and then adding to such bath about three pounds of extract at the beginning of the second week, three pounds at 60 the beginning of the third week, and four pounds at the beginning of the fourth week, the soaking continuing until about the end of the fourth week.

In testimony, that I claim the foregoing 65 as my invention, I affix my signature in presence of two subscribing witnesses this 17th day of October, A. D. 1911.

JAMES C. CLEARY.

Witnesses:

GERTRUDE FALING,  
E. M. KLATCHER.